

## [54] PROCESS FOR CRIMPING POLYESTER FILAMENT YARN

[75] Inventors: **Hans R. E. Frankfort**, Kinston, N.C.; **Peter F. Lyons**, Wilmington, Del.[73] Assignee: **E. I. Du Pont de Nemours and Company**, Wilmington, Del.

[\*] Notice: The portion of the term of this patent subsequent to June 18, 1991, has been disclaimed.

[22] Filed: **May 31, 1974**[21] Appl. No.: **476,129**

## Related U.S. Application Data

[63] Continuation-in-part of Ser. Nos. 281,972, Aug. 18, 1972, and Ser. No. 353,808, April 23, 1973, Pat. No. 3,816,992, which is a continuation-in-part of Ser. No. 210,884, Dec. 22, 1971, abandoned.

[52] U.S. Cl. .... **28/72.17; 57/140 R**[51] Int. Cl.<sup>2</sup> .... **D02J 1/22; D02G 1/16**[58] Field of Search .... **28/72.12, 72.13, 72.17, 28/71.31, 4, 1.2; 264/168; 57/140 R, 140 BY, 140 J, 157 R, 157 F, 157 MS, 34 R, 34 D**

## [56]

## References Cited

## UNITED STATES PATENTS

|           |         |                       |            |
|-----------|---------|-----------------------|------------|
| 2,974,391 | 3/1961  | Speakman et al. ....  | 28/72.13 X |
| 3,115,744 | 12/1963 | Nott.....             | 28/72.17 X |
| 3,226,792 | 1/1966  | Starkie.....          | 28/72.17 X |
| 3,317,978 | 5/1967  | McIntosh et al. ....  | 28/72.17 X |
| 3,358,345 | 12/1967 | Daniel.....           | 28/1.2     |
| 3,379,809 | 4/1968  | Woods.....            | 264/168    |
| 3,816,992 | 6/1974  | Frankfort et al. .... | 28/72.17 X |

Primary Examiner—Louis K. Rimrodt

## [57]

## ABSTRACT

Textile filaments which have asymmetric shrinkage properties, and may be heat-relaxed to provide a high crimp frequency and a narrow crimp frequency distribution, are produced by melt-spinning a single synthetic linear polymer composition, drawing the filaments and then passing them over an unheated wear-resistant pin at high speed. The process conditions are controlled to provide filaments of regular cross-sectional configuration having a modified minor portion, distinguishable from the remainder of the filament by a different refractive index, which extends substantially continuously along the filament.

21 Claims, 3 Drawing Figures



F I G. 1



F I G. 2



FIG. 3



PERCENT OF FILAMENT LENGTH HAVING  
GREATER CRIMP FREQUENCIES

**PROCESS FOR CRIMPING POLYESTER  
FILAMENT YARN**

**REFERENCE TO RELATED APPLICATION**

This is a continuation-in-part of copending applications Ser. No. 281,972, filed Aug. 18, 1972, and Ser. No. 353,808, (now U.S. Pat. No. 3,816,992) filed Apr. 23, 1973. Ser. No. 353,808 is in turn a continuation-in-part of application Ser. No. 210,884, filed Dec. 22, 1971 (now abandoned).

**BACKGROUND OF THE INVENTION**

The present invention is concerned with production of polyester and polyamide filaments which crimp due to asymmetric shrinkage when relaxed.

Filaments which crimp due to asymmetric shrinkage when relaxed have been prepared by a variety of methods. Kilian U.S. Pat. No. 3,050,821 discloses polyester filaments which have been asymmetrically quenched during melt spinning, by blowing cooling air against one side of the filaments as they emerge from the spinneret. When drawn and then relaxed, the filaments will shrink to a greater extent on one side of the filament, but a relatively low crimp frequency is obtained in this manner.

Crimpability has been imparted by passing filaments over a sharp edge. This weakens the filament and improvements in the crimp obtained are desirable. The edge-treated side is on the inside of crimp bends. Terumichi Ono et al. U.S. Pat. No. 3,600,271 discloses that a better crimped product is obtained when previously undrawn 6-nylon is drawn over a cylindrical pin heated to about 600°C. However, Yukio Mitsuishi et al. U.S. Pat. No. 3,538,566 teaches that milder conditions must be used for polyester filaments. Lower pin temperatures are used and the filaments are wet when drawn over the pin in the process of this patent. The results obtained at various pin temperatures and filament speeds of 200 to 600 meters per minute indicate that undesirably low crimp frequencies are obtained.

Edington et al. U.S. Pat. No. 3,224,068 discloses a process in which the treatment is performed after the filaments have been drawn, so that higher temperatures can be used. As illustrated, polyester filaments are passed at speeds of up to 450 yards per minute over a strip of tungsten or tungsten carbide which is about 0.030 inch wide and heated to 365°C.-375°C. Special heating means are used to maintain the strip at an even temperature. The relaxed product is said to have a broad range of crimp amplitudes and crimp frequencies along the filament length, and sections with no crimp at all, but to be an improvement over previous products obtained by treatment with the usual electrically heated wire, pin or bar.

Potman et al. U.S. Pat. No. 3,601,872 discloses that 6-nylon carpet yarn of increased voluminosity can be prepared by introducing two crimps separately into a yarn, a latent crimp by asymmetric treatment with a heated pin and a direct crimp by subjecting the yarn to direct crimping treatment by a gear-crimping, a stuffer-box crimping, or an air-crimping treatment.

**SUMMARY OF THE INVENTION**

The present invention provides for production of multifilament yarns of filaments which, in the heat-relaxed form, have an especially desirable crimp frequency distribution. Additional advantages of the in-

vention will become apparent from the specification and drawings.

The invention is an improvement over previous processes for preparing crimpable yarns by passing a yarn bundle of filaments, spun from a single synthetic linear organic thermoplastic polymer, in contact with a heated surface to provide asymmetric shrinkage properties on opposite sides of filaments. The improvement of the present invention comprises (a) drawing the filaments to provide the approximate break elongation desired in the product and (b) passing the drawn filaments at high speed in frictional contact with a durable, wear-resistant surface under frictional tension sufficient to generate all of the heat required to provide the desired asymmetric shrinkage properties without otherwise heating the wear-resistant surface.

The drawn filaments should be passed in frictional contact with the durable, wear-resistant surface at a speed of at least 900 yards per minute, and more preferably at a speed of at least 2,000 yards per minute. There appears to be no upper limit to the speeds which can be used but speeds within the range of 1,000 to 4,500 yards per minute are generally used.

The yarn filaments must be drawn before the filaments contact the wear-resistant surface in step (b). The drawn filaments preferably have a break elongation of less than 40 percent. Preferably they are drawn so as to have 5 to 25 percent boil-off shrinkage. A preferred process is a coupled spin/draw/pin-texturing process in which the yarn is drawn to have 15 to 40 percent break elongation and 8 to 16 percent boil-off shrinkage prior to contact, in step (b), with a pin having a durable, wear-resistant surface. The temperature of the yarn just prior to the wear-resistant surface should be from 25° to 100°C., although higher temperatures may be used.

The filaments must contact the wear-resistant surface under a frictional tension sufficient to generate all of the heat required to provide the desired asymmetric shrinkage properties without otherwise heating the wear-resistant surface. The term "frictional tension" is used herein to designate the tension on the filaments immediately after the surface minus the tension on the filaments immediately before the surface. Generally, this value is 0.7 to 7 grams per filament; preferably the tension difference is 1 to 2 g./fil. for polyesters and 4 to 5 g./fil. for polyamides.

The filaments usually make frictional contact with the wear-resistant surface for a distance of 0.5 to 15 millimeters. Preferably, the process is operated so that the filaments are in contact with the surface for a distance of 1 to 10 millimeters. Preferably, the durable, wear-resistant surface is provided by a cylindrical pin 3 to 10 millimeters in diameter, but the contact surface can be provided by other means known to the art. The filaments usually contact the surface of the cylindrical pin over an arc of 30° to 180°, and preferably between 45° and 90°.

**BRIEF DESCRIPTION OF THE DRAWINGS**

FIG. 1 is a schematic representation of process and apparatus suitable for continuously melt-spinning drawing and treating filaments in accordance with the invention.

FIG. 2 is a schematic representation of process and apparatus for treating previously drawn yarn in accordance with the invention.

FIG. 3 is a graph of the crimp frequency distribution found in products produced as described in Examples 1 to 5 and then heat-relaxed for 5 minutes in 180°C. air.

## DETAILED DESCRIPTION

In practicing the present invention, the filaments may consist of any single composition of linear organic thermoplastic polymer conventionally used for textile filaments and yarns. The single composition may comprise intimate mixtures of polymers and/or copolymers and may contain minor amounts of other additives, such as delusterants, antistatic agents, or other monomeric or polymeric additives. Polyesters and polyamides are preferred polymers. An especially preferred polyester is polyethylene terephthalate (2GT), as homopolymer or copolymerized with minor amounts of other components. Such copolymerized polyesters include poly(ethylene terephthalate/isophthalate), poly(ethylene terephthalate/adipate) and poly(ethylene terephthalate/5-(sodium sulfo)-isophthalate). Other polyesters include poly(tetramethylene terephthalate) and poly(1,4-cyclohexylenedimethylene terephthalate). Among the polyamide polymers that are preferred are hexamethylene adipamide (nylon 6-6) and the polyamide obtained from bis-(para-aminocyclohexyl) methane and dodecane dioic acid.

The process of the present invention requires that the filaments must be drawn before being treated asymmetrically. Sufficient drawing is necessary to assure that adequate tension conditions can be maintained when the filaments are subsequently passed in frictional contact with the wear-resistant surface. Preferably the drawing is conducted so that the drawn filaments have the approximate break elongation and boil-off shrinkage desired in the product. Usually, it is desired that the break elongation be between 15 and 40 percent, preferably 25 to 35 percent and the boil-off shrinkage be between 5 and 25 percent, preferably 8 to 16 percent.

In the asymmetric treatment step following drawing, the filaments are passed at high speed in frictional contact with a durable, wear-resistant surface. The temperature of the filaments fed to the surface is generally between 25° and 110°C., although higher temperatures may be used. Care should be taken that each filament contacts the surface in approximately the same manner. Preferably, the bundle of filaments is not twisted and the filaments pass over the surface as a single layer of individual filaments. The frictional contact of the filaments with the surface is sufficient to generate enough heat to asymmetrically modify the shrinkage properties of the filaments. No other heating of the wear-resistant surface is necessary.

High speeds are required in the present invention for passing the filaments in frictional contact with the otherwise unheated wear-resistant surface in order to achieve satisfactory asymmetric shrinkage properties in the final product. Usually, filament speeds of at least 900 yards per minute (1,370 cm/sec) are satisfactory, but speeds of at least 2,000 yards per minute (3,050 cm/sec) are preferred. There appears to be no upper limit to the speeds which can be used, but speeds within the range of 1,000 to 4,500 yards per minute (1,525 to 6,860 cm/sec) are generally used.

The tension on the filaments, during passage in frictional contact with the wear-resistant surface, undergoes a distinct change due to the frictional work that is done. This change in tension is equal to tension on the filaments immediately after passage over the surface

minus the tension immediately before passage over the surface. Tension differences of 0.7 to 7 grams per filament are useful, with 1 to 2 g./fil. for polyesters and 4 to 5 g./fil. for polyamides being preferred. These tension differences generally apply to filaments of about 1.5 to 10 denier.

During operation of the process, the filaments usually make frictional contact with the wear-resistant surface for a distance of 0.5 to 15 millimeters, and preferably contact the surface for a distance of 1 to 10 millimeters. Usually the wear-resistant surface is a curved surface, most conveniently provided by a cylindrical pin. Pin diameters of about 1 to 15 millimeters are suitable; 3 to 10 millimeters are preferred. When a cylindrical pin is used, the arc over which the filaments usually contact the pin surface is between 30° to 180°, and preferably between 45° and 90°. Durable, wear-resistant surfaces are needed for satisfactory long-term continuous operation. Ceramic pins of the type commonly used for guides and draw pins in textile processes are suitable. The use of Alsimag, glass and stainless steel pins is illustrated in the Examples. Other metals with durable surfaces are also satisfactory.

To impart asymmetric shrinkage characteristics to any conventional textile filament of synthetic linear organic thermoplastic polymer by means of the process of the present invention, the variables discussed above preferably are adjusted so that the value of  $\Delta T$  max calculated by the following formula is at least 100°C. and usually below 300°C.:

$$\Delta T \text{ max} = 0.0283 (f_2 - f_1) \sqrt{\frac{V}{Lkd}} \quad (1)$$

where  $f_1$  and  $f_2$  are respectively the average tensions on the filaments immediately before and after frictional contact with the wear-resistant surface in grams per filament;  $V$  is the average speed of the filaments contacting the surface in cm./sec.;  $L$  is the frictional contact length between the filaments and the surface in cm.;  $k$  is the thermal conductivity of the filaments in cal./cm.-sec.°C.;  $c$  is the specific heat of the filaments in cal./g.°C.; and  $d$  is the denier per filament. The  $\Delta T$  max parameter is related to the asymmetric temperature distribution that is imposed on the filament by the frictional heat generation and is referred to herein as the "temperature rise parameter."

For conventional polyester textile filaments, the above formula simplifies to the following:

$$\Delta T \text{ max} = 2.26 (f_2 - f_1) \sqrt{\frac{V}{Ld}} \quad (2)$$

For conventional polyamide textile filaments, formula (1) simplifies to the following:

$$\Delta T \text{ max} = 1.92 (f_2 - f_1) \sqrt{\frac{V}{Ld}} \quad (3)$$

Especially preferred operating conditions are obtained in the practice of the present invention when  $\Delta T$  max values of at least 140°C. are used with polyester filaments and of at least 200°C. are used with polyamide filaments.

A continuous process for preparing asymmetrically treated filaments in accordance with the present invention is shown in FIG. 1. Filaments 10 are melt-spun from spinneret 11 and allowed to cool as they descend from the spinneret. The filaments then converge and pass in contact with a conventional first finish-applying roll (not shown). The filaments then proceed around feed rolls 12, through steam draw jet 13, over a second finish-applying roll 14 and then around draw rolls 15, which have a considerably higher surface speed than the feed rolls to draw the yarn. A traversing mechanism 16 is provided for guiding the filaments onto the draw rolls. When activated, the mechanism 16 varies the path of the drawn filaments on the rolls and over a wear-resistant pin 17, which is referred to herein as a "texturing pin." It is at pin 17 that the asymmetric treatment of the filaments occurs. The drawn filaments pass over texturing pin 17 with a change of direction  $\theta$ , and pass around pulling rolls 18 which provide tension over the texturing pin 17. If desired, the filaments can be guided to the texturing pin by an adjustable idler roll (not shown) to facilitate changing the wrap angle  $\theta$  at the texturing pin in order to increase or decrease the length of pin-filament contact. The filaments pass from the pulling rolls 18 over a postdraw finish roll 19 to wind-up 20, which cross-winds the product under a tension that is best measured shortly after the postdraw finish roll.

In operating the process of the present invention, normal levels of finish, such as are typically used in spinning-drawing-winding operations, are used. Excess finish should be avoided so as not to have it interfere with frictional work at the pin-filament contact site.

Crimp is developed in the above product by a subsequent heat relaxation treatment. However, the processes may be combined to produce a crimped product in one continuous operation. Instead of wind-up 20, the filaments may be passed through heating means on a conveyor in relaxed condition and then cooled prior to being wound up. On the other hand, the melt-spinning, drawing and pin-texturing sequence can be split in various ways. The melt-spinning can be a separate operation. A conventional melt-spinning and drawing process can be used to produce yarn which is later pin-textured in a separate operation.

FIG. 2 illustrates such a separate operation wherein untwisted, drawn and packaged yarn is fed over-end to the pin-texturing treatment. The yarn passes from package 21 through tension gate 22 and over roller 23 to a pair of feed rolls 24. The yarn makes several wraps about the pair of feed rolls, proceeds to a pair of stretch rolls 25, makes several wraps about the pair of stretch rolls, passes over texturing pin 26 at a wrap angle  $\theta$ , and proceeds over roller 27 to wind-up 28. The yarn passing over the texturing pin may be an inner wrap, i.e., the yarn passes from the pin back to the stretch rolls. Alternatively, the yarn may pass from the pin to separate pulling rolls without returning to the stretch rolls.

In the pin-texturing portion of the above-described processes, wherein the filaments are fed to the frictional contact surface (e.g., a pin) by feed rolls and withdrawn therefrom by takeup rolls, the filaments usually are stretched by no more than 10 percent, and preferably by no more than 5 percent. When operating the invention with a process in which the melt-spinning and drawing are separated from the pin-texturing step, a stretch of substantially zero (i.e., no stretching) can be used satisfactorily in the pin-texturing step. With

polyester yarns in a continuous process, it is preferred to operate with a stretch of between 2 and 5 percent.

The multifilament yarns produced in accordance with the above-described processes of the invention may be of any conventional denier/filament count. Generally, yarns of about 35 to 250 denier having 10 to 200 filaments are suitable. Yarns having 17 to 50 filaments are preferred. Yarn counts of 70/34 to 190/34 are especially preferred. Filament deniers of 1.5-10 are suitable, but 2-5 are preferred.

Crimp may be developed in the yarns produced according to the invention by any of the many well-known conventional heat-relaxation treatments. In general, these treatments allow the yarn to shrink freely while exposed to hot water, steam or dry heat. In the method used herein for comparing the crimp frequencies of filaments, the filaments are suspended free of tension in an oven through which hot air at 180°C. is gently circulated for five minutes and then the filaments are allowed to cool while still free from tension. Filaments which have been relaxed by other methods are also retreated by this test method to standardize crimp measurements.

The process of the present invention also provides a particularly useful, novel polyester filament which when heat-relaxed has an especially desirable crimp frequency distribution. Yarns made of such filaments have additional advantages in use, which will be discussed below. This product of the invention is a textile filament having asymmetric properties and an abraded surface extending along one side of the filament, and consisting of a single synthetic linear polyester composition. The filament has a modified minor portion distinguishable by a difference in refractive index, which extends substantially continuously along the abraded side of the filament. The continuity of this minor portion is such that less than 5 percent, preferably less than 3 percent, of the filament length is occupied by discontinuities longer than 2 millimeters and the average length of all discontinuities is less than 2 millimeters, preferably less than 1.5 mm. The number of discontinuities longer than 2 mm. is usually less than 30 percent of the total number of all discontinuities and is preferably less than 15 percent. In general, the minor portion occupies 3 to 20 percent, preferably 4 to 15 percent, of representative cross-sectional areas along the filament and is usually 1 to 3 microns, preferably 1.4 to 2.6  $\mu$ , in thickness, measured from the abraded surface. The filament is capable of crimping when given a heat-relaxation treatment for 5 minutes in air at 180°C. The abraded surface of the filament is generally on the outside of crimp bends and is marked by closely spaced, parallel ripples which extend transversely with respect to the filament length. These ripples are clearly visible when the filament is viewed under high magnification.

A heat-relaxed product of the invention is as defined above and further characterized by crimp frequency values, measured after a heat-relaxing treatment for 5 minutes in 180°C. air and normalized for 2.5 denier per filament, which average at least 10, preferably 25 to 60, crimps per filament inch with a percent coefficient of variation of less than 30, preferably less than 20. Preferably at least 95 percent of the filament length has greater than 15 crimps per filament inch and the crimp frequency distribution for the middle 90 percent is numerically equal to or less than said average (usually from 0.4 to 0.9 times the average crimp frequency value). Preferably at least 90 percent of the filament

length has greater than 20 crimps per inch.

Crimp frequencies are expressed herein as crimps per filament inch, rather than crimps per straight line inch of crimped length. The measurement is accomplished by extending the filament under a load sufficient to straighten the crimps without stretching the filament, marking 1-inch (2.54 cm.) distances along the filament, then removing the load to allow recrimping, and counting the crimps between 1-inch (2.54 cm.) marks. In order to compare filaments of different deniers, the measured crimp frequency values are multiplied by  $\sqrt{d/2.5}$ , where  $d$  is the denier per filament after 180°C. treatment, to obtain normalized crimp frequency values. If the percent shrinkage ( $S$ ) in the 180°C. oven-relaxing treatment is known, the value of  $d$  can be determined by multiplying the unrelaxed denier per filament by  $(1 + S/100)$ .

A characteristic abraded surface, which extends substantially continuously along one side of the filaments of this invention, provides a qualitative distinction from prior art filaments that have been modified in different ways to impart crimp. The location of modified filament portions in heat-relaxed filaments is indicated by closely spaced, parallel ripples crossing the filaments. FIG. 3 shows the crimp frequency distributions of products produced as described in Example I below and then heat-relaxed for 5 minutes in 180°C. air. The normalized crimp frequency in crimps per filament inch is indicated on the abscissa, and the percent of the filament length having greater crimp frequencies is indicated on the ordinate. The distribution curves are numbered to correspond to yarn numbers. The graph can be used to ascertain the percent of the filament length which has a crimp frequency greater than any given value. The average crimp frequency is the value where the 50 percent ordinate value intersects the curve. The crimp frequency distribution for the middle 90 percent is the minimum crimp frequency for 5 minus the minimum crimp frequency for 95 percent; which will be abbreviated  $R_5 - R_{95}$ .

Woven and knit fabrics containing relaxed yarns of this invention have desirable bulk aesthetics, performance and uniformity. For example, yarns of the type described in Example I-3 below, when relaxed in a hot air jet and then woven into fabrics, yield fabrics that have a high degree of suppleness and liveliness; warp-knits from similarly relaxed yarns have a soft hand, high bulk, and excellent dye-uniformity. Double-knit fabrics prepared from relaxed yarns of Example I, yarn sample 2, have a high, firm bulk and excellent wash-wear performance, wrinkle-resistance, and dye-uniformity. Suitable filaments for such yarns are between 1 and 7 denier per filament. The yarns of the present invention can also be cut into staple lengths and converted to yarns or used as filling, as in pillows, after developing the crimp.

#### EVALUATION PROCEDURES

##### Photomicrographs of Filament Surfaces

A scanning electron microscope is used to examine the nature of the abraded surface of the filaments. A short sample (about 1.9 cm. long) of yarn is mounted on a standard "Stereoscan" stub (1.9 cm. diameter aluminum stub). Two strips (0.32-cm.  $\times$  0.63-cm.) of double-faced adhesive tape are fixed 1.27-cm. apart and parallel to each other on the stub surface. The sample of yarn is lightly teased to separate the filaments, and

each yarn end is fixed to one strip of the adhesive. When mounting crimped yarn, no tension is applied so that the yarn is mounted with its crimp undisturbed. Silver circuit paint is dabbed on both ends of all filaments and on the adhesive tape to insure electrical continuity to the specimen stub. The final step of specimen preparation involves the vacuum evaporation of a 60/40 Au/Pd coating onto the surface of the sample and stub which insures electrical continuity over the entire stub. The thickness of this coating is estimated to be of the order of 300-400 Å which is below the level of resolution of the scanning electron microscope used; thus, the coating is not seen when viewing filaments by this technique.

The stub is placed in the specimen holder and after evacuation of the specimen chamber, the specimen is viewed in the scanning electron microscope. Typical viewing conditions are 20 KV electrons with a beam current of 200  $\mu$ amps, and a specimen tilt of 30° relative to the impinging electron beam. After areas of the filaments exhibiting modified surfaces are located, photomicrographs are recorded at, e.g., 200, 500, 1,000 and 2,000 $\times$  magnifications. This series of magnifications includes a sufficiently low magnification to illustrate the position of the modified surface relative to the crimp and a sufficiently high magnification to reveal details of the modified surface.

When viewed by this technique, unrelaxed filaments of the present invention exhibit a frictionally modified surface running along the filament length; in the relaxed filaments, this surface can be seen to be present along the outside of the crimp bend and can also be seen to have a plurality of ripples. These ripples are visible on the abraded surface and run transverse to the filament length. In the relaxed filaments that have been jet-screen treated (e.g., as in Example II below), the modified surface also runs generally on the outside of crimp bends, but may occasionally be seen on the inside where secondary folds have been imposed on sections of the filament by jet-screen impact.

##### Continuity of the Modified Portion

Interference microscopy is used to determine the continuity of the modified portion along filament length "Z", where Z is taken as 40 mm. times the number of filaments in the yarn for any yarn having 34 filaments. For other yarn counts, a total of 1,360 mm., distributed uniformly across the yarn, is viewed.

When working with a 34-filament yarn, a 60 mm. length is cut from the yarn. The individual filaments are separated. Each 60-mm. long filament is taped on a glass slide so that it lies straight. The slide is immersed in Refractive Index Fluid of an index of refraction ( $n$ ) which matches the index of refraction ( $n$  perpendicular) of the unmodified portion of the filament for light vibrating perpendicular to the fiber axis (e.g., a fluid of  $n = 1.540$  is used for polyethylene terephthalate). The filament, after immersion in the fluid, is then covered with a second glass slide and the assembly is placed on the stage of the interference microscope. The assembly is advanced across the viewing area so that a continuous 40 mm.-length is viewed at 200 $\times$ .

The presence of a modified portion is detected by interference contrast (i.e., the modified portion will be of different color than the remainder of the filament) or by fringe field (i.e., a fringe shift indicates a change in index of refraction going from modified to unmodified areas of the filament). Only those sections where a

color difference or a fringe shift can be positively identified are considered as modified. Once a modified portion is detected, its path is followed along the filament length and the number and length of all discontinuities in its path are recorded. For convenience, a calibrated eyepiece, such that at 200 $\times$  each division on the eyepiece equals 5 $\mu$ , is used and the length of the discontinuities is reported in "divisions" and later converted to mm. by the formula:

$$\text{mm.} = \left( \frac{\text{number of divisions}}{1000} \right) \times 5$$

The following are determined:

- M = total number of all discontinuities  
 N = number of discontinuities greater than 2 mm. (2  
     mm. = 400 divisions)  
 U = sum of the lengths of all discontinuities, expressed  
     in mm.  
 W = sum of the lengths of discontinuities greater than  
     2 mm., expressed in mm.  
 Z = total filament length viewed

From these values, the following are calculated:

- Average length of all discontinuities = U/M  
 % of long (>2 mm.) discontinuities = (N/M)  $\times$  100  
 % of filament length occupied by long (>2 mm.) dis-  
 continuities = (W/Z)  $\times$  100

The products of the present invention have a low average length for all discontinuities, and the long discontinuities, if present, occupy only a very minor portion of the total length of the filament. It is believed that these factors contribute significantly to the desirable crimp of the products, since the presence of the modified portion correlates well with the development of crimp in the filaments.

#### Dimensions of Modified Portion: Cross-Sectional Views

A cross-section of the yarn sample is suitably prepared for microtome sectioning, e.g., a yarn bundle is mounted in a "Beem" capsule and embedded with epoxy ("Maraset" from Marblette Corp.). After trimming the cured stub, approximately 6 micron thick sections are obtained using a rotary microtome (Spencer Model 860) with a steel blade. The sections are placed onto the two halves of a cut microscope slide (insures constant thickness for a two beam Leitz Transmission Interference Microscope). The "two" specimen slides are completed by immersing the sections in refractive index oil (Cargille Index of Refraction Fluid N = 1.530) and covering with microscope cover slips.

One specimen slide is placed onto the reference beam stage and the other slide is placed onto the sample beam stage of the two beam Leitz Transmission Interference Microscope. The specimen section is viewed at 500 $\times$  magnification. Following the alignment procedures, the fringe field is obtained in the field of view in white light. The fringes are then "fluffed out" to obtain interference contrast, i.e., the fringes are taken to their maximum separation. The specimen section is brought into sharp focus and the index variation across the textured filament cross-section is recorded on color film as

the retardation or color difference across the filament section. The procedure can be carried out in monochromatic illumination and recorded on black and white film. The procedure described above is performed without the analyzer in the optical system and is used as a qualitative detection technique for presence of the modified portion of different refractive index.

Thickness of the modified portion is determined from 1,000 $\times$  micrographs of cross-sections by measuring 10 with a ruler the thickness on three cross-sections at three points each, and averaging the nine values. In these measurements 1 mm. = 1 $\mu$ . The three points measured on the photomicrograph are (1) the thickness at the center of the modified portion and (2) and 15 (3) the thickness near each of the extremes of the modified portion, measured at a distance of about 1 mm. from each extreme.

The width of the modified portion at its widest point and the diameter of the filament are also measured on 20 1,000 $\times$  micrographs of cross-sections. Four or five cross-sections per sample are analyzed and the average of the four or five determinations is recorded.

The % area of the modified portion is determined by 25 making a 1,000 $\times$  photomicrograph, cutting out 8-12 cross-sections from it, and weighing these cross-sections before (W<sub>B</sub>) and after (W<sub>A</sub>) cutting the modified portion therefrom. % Area = (W<sub>B</sub> - W<sub>A</sub>) (100/W<sub>B</sub>) when W<sub>B</sub> and W<sub>A</sub> are total weights in grams, before and after cutting.

#### Crimp Frequency Distribution

For a yarn having at least 17 filaments, a 50-cm. length of yarn is cut from the yarn to be tested, and 35 17 filaments, taken at random, are carefully separated from the cut length, taking care not to stretch the filaments. One filament at a time is relaxed as follows: The filament is suspended by attaching both ends to a glass rod at a sufficient distance apart to permit the filament to shrink and crimp fully without becoming taut; this is done, e.g., by attaching masking tape or a suitable clip to each end of the filament and clipping each end to the rod. The rod may be permanently mounted in the oven or placed in the oven, with the filament already attached to it. Hot air at 180°C. is gently circulated in the oven for 5 minutes by the oven blower, which is set at minimum to avoid filament entanglement. A suitable oven for this test is Electric Hotpack Co., Inc., Model 1354. The thusly suspended filament is free to relax. Then, taking care not to stretch the filament, the filament is removed from the oven and is carefully placed in a relaxed condition on a velvet board. After removal of each specimen, the oven is allowed to come back to 180°C. (e.g., 5 minutes) before the next specimen is placed in the oven. This is repeated until all 17 filaments have been relaxed, individually.

One end of each relaxed filament is then taped to one end of a clear plastic straight-edge which is marked in 1-inch (2.54 cm.) intervals. A weight, sufficient to straighten the crimps without stretching the filament, is 60 taped to the free end of the filament. For example, a 0.6 g. weight is normally satisfactory for filaments of about 2 to 6 dpf. The straight-edge is lifted to a vertical position, allowing the filament to hang freely under the tensioning weight. The filament is then taped to the 65 straight-edge near the weighted end, while under tension. With a black felt-tipped marking pen, twelve consecutive 1-inch sections are marked off on the filament. The filament is then removed and taped at its ends, re-

laxed, on a second, clear straight-edge. The markings on the filament are duplicated on the second straight-edge along side of the filament with a black felt pen. This allows direct measurement of the crimps per filament inch. The number of crimps between the markings are counted at about  $20 \times$  magnification using a shadowgraph (e.g., Nippon Kogaku K.K., Japan, Model 6). Crimps per each filament inch (cpi) for a total of 204 one-inch filament sections per sample are recorded (17 filaments  $\times$  12 one-inch sections).

If the yarn contains less than 17 filaments total, a sufficient length of yarn is used, so that the number of filaments times the length equals 204 inches (518-cm.).

The number of one-inch sections in each of a series of crimp ranges (0-5 cpi, 6-10 cpi, 11-15 cpi, etc., in increments of 5 cpi/range) is counted and the percent of filament length within a given crimp range is calculated by:

$$\frac{\text{Number of 1-inch sections in given crimp range}}{204 \text{ sections}} \times 100$$

Data are reported in terms of % filament length present, having a crimp frequency greater than a given level, using as levels the upper limit of each crimp frequency range, i.e., > 5 cpi, > 10 cpi, > 15 cpi, etc. The respective observed crimp frequency values are multiplied by  $\sqrt{d/2.5}$  to obtain normalized crimp frequency values, where  $d$  is the denier per filament after the heat-relaxing treatment in 180°C. air for 5 minutes. Any accurate method can be used for determining  $d$ . The method used herein is to multiply the denier per filament before the heat-relaxing treatment by  $(1 + \frac{S}{100})$ , where  $S$  is the percent shrinkage calculated from yarn lengths before and after the heat-relaxing treatment when measured under sufficient tension to just straighten any crimps without stretching the yarn (a tension of 20 grams is suitable for 34-filament yarns in the Examples unless otherwise specified).

Illustrative data for one of the examples (i.e., Ex. 1, yarn 2) is given below:

| Crimp Range at d dpf (cpi) | No. of 1-inch Sections | % Filament Length Present |
|----------------------------|------------------------|---------------------------|
| 0-5                        | 0                      | 0                         |
| 6-10                       | 0                      | 0                         |
| 11-15                      | 0                      | 0                         |
| 16-20                      | 0                      | 0                         |
| 21-25                      | 1                      | 0.5                       |
| 26-30                      | 15                     | 7.3                       |
| 31-35                      | 56                     | 27.4                      |
| 36-40                      | 73                     | 35.7                      |
| 41-45                      | 48                     | 23.5                      |
| 46-50                      | 11                     | 5.4                       |

The above data may be expressed as follows:

| Crimp Level at d dpf                           | Crimp Level (Normalized for 2.5 dpf) |
|------------------------------------------------|--------------------------------------|
| 100% Filament length with crimp frequency 100% | > 5 cpi                              |
| 100%                                           | > 10 cpi                             |
| 100%                                           | > 15 cpi                             |
| 100%                                           | > 20 cpi                             |
| 99%                                            | > 25 cpi                             |
| 92%                                            | > 30 cpi                             |
| 65%                                            | > 35 cpi                             |
| 29%                                            | > 40 cpi                             |
| 5%                                             | > 45 cpi                             |

-continued

| 5 | Crimp Level at d dpf | Crimp Level (Normalized for 2.5 dpf) |
|---|----------------------|--------------------------------------|
|   | 0%                   | > 50 cpi                             |

The above determined data are plotted on a graph as "% filament length with crimp frequency greater than" vs. "crimp frequency level, normalized for 2.5 dpf". This graph can then be used to ascertain % filament length with crimp frequency greater than any given value of crimp frequency.

The crimp frequency distribution for the middle 90 percent is defined as  $R_5-R_{95}$ , where  $R_5$  is the value read from the graph at the 5 percent level and  $R_{95}$  is the value read at the 95 percent level. For a narrow crimp frequency distribution, the ratio of  $R_5-R_{95}$  to the average crimp frequency is equal to or less than 1.

The percent coefficient of variation is defined as the standard deviation of the individual determinations of crimp frequency ( $F$ ), times 100 and divided by the average crimp frequency in crimps per inch. The standard deviation is calculated by the formula:

$$\text{Standard deviation} = \sqrt{\frac{\sum F^2}{N} - \left[ \frac{\sum F}{N} \right]^2}$$

where  $N$  is the number of determinations. A percent coefficient of variation which is less than 30 indicates a narrow crimp frequency distribution and a value less than 20 indicates a highly uniform crimp.

In the Examples unless otherwise specified, a yarn finish is applied by conventional means (i.e., 1st and 2nd finish-applying rolls referred to in the discussion of FIG. 1). This finish, referred to hereinafter as finish "A", is a 3.9 percent aqueous mixture containing 49 parts of isocetyl stearate, 24.5 parts of sodium di-(2-ethyl-hexyl)sulfosuccinate, 24.5 parts of the condensation product of 1 mol of stearyl alcohol with 3 mols of ethylene oxide, 1 part of triethanolamine and 1 part of oleic acid. The total amount of finish applied to the filaments is approximately  $0.3 \pm 0.1$  weight percent finish on yarn after drying, based on the weight of yarn.

Just before wind-up, (e.g., at roll 19 of FIG. 1) the yarn is treated with another conventional finish (noted hereinafter as finish "B") which is an aqueous mixture containing 20.5 parts of sulfated peanut oil, 1.8 parts of diethylene glycol, 1.8 parts of KOH, 62.6 parts of the ester formed from 1-butanol and a 45-55 mixture of stearic and palmitic acids, 8.2 parts of oleic acid, 3.4 parts of triethanolamine, and 1.7 parts of ortho phenylphenol. This second finish is applied to give a total of A plus B of about  $0.5 \pm 0.15$  percent finish on the yarn after drying.

In the Examples, the process of the invention is illustrated with yarns having filaments of circular cross-section, although the process may operate satisfactorily with yarns of other cross-sections as well. Break elongation and boil-off shrinkage are measured on filaments before or after pin-texturing: break elongation by ASTM-D-2256-69; and boil-off shrinkage by comparing filament length before and after 30 minutes exposure in boiling water. Unless otherwise specified, yarn tension is measured with a Schmidt-Waldkraiburg tensiometer (0-1000 gram scale).

Different texturing pins are used in the examples. These are identified as follows:

- Type 1 — White Alsimag 614 having a matte finish and measuring  $\frac{1}{16}$ -inch (0.95 cm.) in diameter (such pins having a smooth finish are referred to as Type 1a);  
 Type 2 — Brown Alsimag 586 having a smooth finish and measuring  $\frac{3}{16}$ -inch (0.48 cm.) in diameter;  
 Type 3 — Cream colored Alsimag 192 having a smooth finish and measuring  $\frac{1}{16}$ -inch (0.95 cm.) in diameter;  
 Type 4 — Stainless steel 304 having a  $\frac{1}{4}$ -inch (0.63 cm.) diameter;  
 Type 5 — Glass rod of  $\frac{1}{4}$ -inch (0.63 cm.) diameter.

Some typical thermal conductivities and coefficients of friction (measured by the technique described by J. S. Olsen, "Frictional Behavior of Textile Yarns," *Textile Research Journal*, Vol. 39, No. 1, Jan., 1969, using a 6-gram input tension and a 500-*yd./min.* [457 meters/min.] speed) for these pins are:

| Type | Thermal Conductivity<br>(cal./cm.sec.°C.) | Coefficient<br>of friction |
|------|-------------------------------------------|----------------------------|
| 1a   | $0.124 \times 10^{-4}$                    | 0.48                       |
| 3    | $0.41 \times 10^{-3}$                     | 0.56                       |
| 4    | 0.124                                     | 0.82                       |

Alsimag is a registered trademark in the U.S. for pressed and extruded steatite thread guides, beryllia ceramics, and leachable ceramic cores. Steatite is a mixture of clay, talc and alkaline earth oxides. The Alsimag pins used in the Examples are made by American Lava Corp. of Chattanooga, Tenn. Pins having friction coefficients of 0.2-1.2 are suitable for use in the invention; coefficients of 0.4-0.8 are preferred.

#### EXAMPLE I

This Example illustrates the production of six polyester yarns in accordance with the present invention. Process conditions are summarized in Table I. The crimp characteristics of the resultant yarns are presented in Table II. Crimp frequency distributions for the first five yarns are plotted in FIG. 3.

All of the yarns of this example, except yarn 5 are prepared by a continuous process in which polyethylene terephthalate polymer is melt-spun, drawn and pin-textured as shown in FIG. 1. The process for yarn 5, illustrated in FIG. 2, involves the use of previously melt-spun, drawn and packaged commercial semi-dull polyethylene terephthalate filaments. These yarn-5 filaments, prior to pin texturing, formed a 34-filament, 70 denier yarn having a boil-off shrinkage of about 10 percent and a break elongation of about 36 percent. Finishes A and B were applied to yarn 5 prior to pin texturing, as described above. In the pin texturing of yarn 5, per FIG. 2, an inner wrap of yarn, lifted from the stretch rolls 25, passes over the texturing pin 26 and back around the stretch rolls before the yarn continues to the wind-up 28. Yarns 3 & 4 illustrate the use of very short contact lengths on the texturing pin. Yarn 6 illustrates the use of relatively low viscosity filaments. All polyester relative viscosities listed in Table I and subsequent tables are measured at 25°C. in a solution of 8 grams of polymer in 100ml. of hexafluoroisopropanol containing 100 parts per million of sulfuric acid.

In the drawing steps for yarns 1 through 4 and 6, the draw rolls are located in a temperature-controlled en-

closure, called a "draw box." Since the filaments in this example lose very little heat in traveling from the draw box to the texturing pin, the yarn temperature at the feed pin is listed in Table I as being at the same temperature as the draw box.

- Yarn 2, which as indicated in Table I, is produced in a similar manner to yarn 1, but is further processed by a jet-screen-bulking step. After pin-texturing, the yarn is fed at about 3000 yards/minute (2740 meters/minute) at a temperature of about 125°C. to a hot-air jet device which deposits the yarn on a screen drum as illustrated in Clendening U.S. Pat. No. 3,217,386. The jet device is of the type disclosed in Coon U.S. Pat. No. 3,525,134 and is supplied with hot air at 335°C. and 100 pounds per square inch (7kg/cm<sup>2</sup>) gauge pressure. The jet device comprises a longitudinal yarn passage terminating in a short length having a width  $d_t$  of 0.033-inch (0.085 cm.) and a depth of 0.030-inch (0.076 cm.); a throat region having a width  $d_t$  of 0.045-inch (0.114 cm.); an expanding treatment chamber whose sides diverge at an angle  $\beta$  of 4.5° from the throat region to a width  $d_e$  of 0.22-inch (0.56 cm.) at the chamber exit; and dual fluid conduits, each having a width  $d_o$  of 0.025-inch (0.064 cm.), disposed on either side of 20 the yarn passage and intersecting the throat region at an angle  $\alpha$  of 30°. The dual fluid conduits and the yarn treatment chamber have the same depth of 0.060-inch (0.152 cm.).

The heated air supplied to the jet device forwards the 30 yarn through the treatment chamber, plasticizes it and propels it against a screen surface on a rotating relaxing drum. The screen drum surface is of 40-mesh, located 0.050-inch (0.127 cm.) from the jet exit and revolving at 700 feet per minute (213 meters/minute). Residence time on the drum is 0.12 second. The treated yarn is taken from the screen drum at about 2,220 yards per minute (2,010 meters/minute) by a pair of rolls and proceeds at 20 grams tension to a wind-up for packaging. Table II lists the properties and FIG. 3 shows the crimp frequency distribution of the final product (i.e., the pin-textured product that has also been jet screen bulked).

#### EXAMPLE II

This example describes another embodiment of the invention in which polyester filaments which have been melt-spun at relatively high speeds are pin-textured and then jet-screen bulked. Process conditions for the drawing and pin-texturing steps are given below and in Table I. The crimp characteristics of the final product are summarized in Table II.

Polyethylene terephthalate of 19.5 relative viscosity and containing about 0.3 percent, by weight, of TiO<sub>2</sub> delusterant is melt-spun at 284°C. through a spinneret 55 having 34 round holes, each hole having a diameter of 0.011-inch (0.028 cm.) and a length of 0.020-inch (0.051 cm.). The freshly spun filaments are quenched with air at 23°C. in crossflow against the filaments and then passed through a guide, past a finish roll to a pair 60 of puller rolls, situated 188 inches (4.78 meters) below the spinneret and revolving at a peripheral speed of 3,398 ypm (3,107 meters/minute). The yarn wraps around these rolls and, subsequently, passes around rolls moving at 3,403, 3,409, and 3,413 ypm, (3,112, 3,117, and 3,121 meters/minutes) respectively, which maintain tension on the yarn. The yarn then passes through an interlace jet and to a second finish roll and is then wound up at 3,411 yards per minute (3,119 me-

ters/minute) to form a package.

The interlace jet is of the type described in Bunting et al. U.S. Pat. No. 3,115,691. The interlace jet produces an interlace pin count, as measured according to Hitt U.S. Pat. No. 3,290,932, of about 20 cm.

Finish is applied at first and second finish rolls in an amount of 0.50 percent, based on the weight of the fiber. The finish is of the general type described in U.S. Pat. No. 3,594,200 to Cooley and Finch. Its composition is as follows: 28 parts of coconut glycerides, 37 parts (on a wet basis) of sulfated peanut glycerides having a 20 percent water content, 25 parts of Gafac PE-510, i.e., an acid phosphate of ethoxylated nonylphenol as depicted by the formula at Col. 2, line 5 of U.S. Pat. No. 3,594,200, and 10 parts of Shell 277 (a mixture of paraffinic and alicyclic hydrocarbons). To this mixture is added enough 45% KOH to give a pH of 6.5.

The yarn obtained in this fashion is a 247 denier-34-filament yarn having a tensile strength of 2.47 grams per denier, an elongation of 129.1 percent, and an initial modulus of 30.94 grams per denier. An X-ray pattern of the yarn shows that it is amorphous, having no measurable crystallinity. The orientation angle is 14° and the density of the filaments is 1.342 grams per cc.

The as-spun yarn from its package is then led to a pair of feed rolls rotating at a peripheral speed of 668 yards per minute (611 meters/min.) making 7-8 wraps about the rolls then passed in sliding contact with ice cold metal finish roll rotating in an ice/water bath. From the finish roll the cooled yarn travels a distance of less than about 8 inches to a T-pipe having a yarn passageway with a diameter of  $\frac{5}{8}$ -inch (1.59 cm.) and length of 10 inches (25.4 cm.) into which atmospheric steam is fed. As the yarn passes through the pipe, it is subjected to the 95°-100°C. mixture of hot water and atmospheric steam in the pipe. Steam exits from the pipe at the entrance and exit of the yarn passageway. From the pipe, the yarn passes a distance of less than about 8 inches (20.3 cm.) to a second ice cold metal finish roll rotating in bath containing a mixture of ice and water. The cooled yarn then passes to a pair of draw rolls rotating at a peripheral speed of 1,499 yards per minute, (1371 meters/min.) making 8-9 wraps about the rolls. In its passage from the feed rolls to the draw rolls, the yarn is drawn 1.94X. The drawn yarn has an elongation of about 13-14 percent. The yarn then passes from the draw rolls over a Type 3 unheated AlSiMag 192 texturing pin. The AlSiMag pin is stationary and the yarn passes over it in frictional contact with it at an angle of 90°. From the pin the yarn passes to rolls rotating at a speed of 1,518 yards per minute (1,388 meters/min.) making 5-6 wraps about the rolls and then to a package.

Tension on the yarn during drawing, as measured with a Schmidt-Waldkraiburg tension measuring device inserted in the running line, is 190 grams. Yarn tension measured in the same way before and after the pin is 50-90 grams (before) 200-230 grams (after). The calculated  $\Delta T$  max parameter for this process is 273°C.

The properties determined on the pin-treated yarn are as follows:

|                                   |       |
|-----------------------------------|-------|
| Density (grams per cc):           | 1.364 |
| Denier:                           | 130   |
| Tenacity (gpd):                   | 4.42  |
| Elongation (%):                   | 13.6  |
| Modulus (grams per denier)        | 98.14 |
| Yield Tenacity (grams per denier) | 1.35  |

-continued

Crystallinity Index: 27-28  
Orientation Angle: 14-16°

5 The yarn is then unwound from a package and subjected to a jet/screen relaxing treatment under the following conditions: The yarn is led to a set of feed rolls rotating at a peripheral speed of 1,455 yards per minute, (1,330 meters/min.) making 12 wraps about the feed rolls. From the feed rolls the yarn passes into a jet.

10 The jet device used is of the type described in Yngve U.S. Pat. No. 3,638,291. Referring to FIG. 2 of the Yngve patent, the dimensions of the jet are as follows:

15

|                                                                          | Inches         | cm.            |
|--------------------------------------------------------------------------|----------------|----------------|
| Diameter of Internal Supply Manifold 22                                  | 0.1906         | 0.4841         |
| Dimensions of Angularly Disposed Conduits, 24,26                         |                |                |
| (width)                                                                  | 0.0405         | 0.1029         |
| (length)                                                                 | 0.2595         | 0.6591         |
| Width of Yarn Passage Section 34                                         | 0.042          | 0.107          |
| Depth of Enlarged Throat Region 36                                       | 0.030          | 0.076          |
| Depth of Triangular-Shaped Expansion Cavity 38                           | 0.059 to 0.060 | 0.150 to 0.152 |
| Width of Opening 39                                                      | 0.1073         | 0.2725         |
| Included Angle of Continuously Expanding Treatment Chamber 40 in degrees | 6              |                |

20 The jet is supplied with steam at 25 to 28 psi (1.76 to 1.97 kg/cm<sup>2</sup>) gauge and 300° to 305°C. From the jet the yarn is impacted against a screen mounted on drum moving at a peripheral speed of 7 yards per minute (6.4 meters/min.), the drum being a 3½-inches (8.9-cm.) wide, 15-inch (38.1-cm.) diameter drum having a 60-mesh screen on its surface. An accumulated mass of 25 yarn travels for a distance of about 15 inches (38.1 cm.) along the drum circumference. From the drum the yarn passes over guide rolls to a wind-up where it is wound up at about 1,100 yards per minute (1,006 meters/min.). The untwisted yarn has the following properties:

|    |                              |        |
|----|------------------------------|--------|
| 45 | Tensile Strength (gpd)       | 3.65   |
|    | Elongation                   | 37.91% |
|    | Modulus (gpd)                | 14.8   |
|    | Denier                       | 165    |
|    | Yield Tenacity (gpd)         | 0.77   |
|    | Average Density (g. per cc.) | 1.392  |
|    | Crystallinity Index          | 63%    |
|    | Orientation Angle            | 25°    |

50

Additional properties are given in Table II.

A sample of the yarn is then knit into a Swiss-pique fabric (18-cut). The fabric has good bulk and desirable hand, texture and appearance.

55

### EXAMPLE III

This example illustrates pin-texturing of polyester filaments in five continuous high speed process embodiments of the invention, in which several process parameters were varied; for example, pin composition, texturing speed from 1,300 to 2,800 yards/minute (1,189 to 2,560 meters/min.) and pin contact length. This series of runs, along with those of the other examples and numerous other data, were useful in developing the  $\Delta T$  max parameter for defining preferred operating conditions of the invention.

60 In each of runs A through E, polyethylene terephthalate polymer of 22.0 relative viscosity and containing

0.3 weight percent titanium dioxide was melt-spun into 34 round filaments, which are then passed through a jet operating at 225°C. and 85 psi (6 kg/cm<sup>2</sup>) gauge. The drawing conditions, as well as the details of the pin-texturing step are summarized in Table III. The tensions are measured with a Rothchild Tensiometer having rolling guides with high speed bearings on the tension head, using the 0 to 1000-gram tension range. The apparatus arrangement of FIG. 1 is used. Characteristics of the pin-textured yarns are given in Table IV.

|                      | Yarn A<br>6-6 Nylon | Yarn B<br>PACM-12 |
|----------------------|---------------------|-------------------|
| Tenacity(gpd.)       | 5.6                 | 3.5               |
| Elongation(%)        | 22                  | 24                |
| Modulus(gpd.)        | 31                  | 35                |
| Denier               | 130                 | 227               |
| Density              | 1.1295              | 1.0802            |
| Orientation Angle(°) | 16                  | 32                |
| Crystallinity Index  | 48                  | <5                |

#### EXAMPLE IV

This example illustrates the process of the invention with two types of multifilament polyamide yarns. Yarn A is Zytel 101, made from polyhexamethylene adipamide (6-6 nylon) of 45 relative viscosity. Yarn B is made from the polyamide, called PACM-12, which is obtained from bis-(para-aminocyclohexyl)methane and dodecane dioic acid. The filaments are pin textured on unheated glass rods (Type 5).

Each polyamide yarn is spun, drawn and wound up before being pin textured. Properties of typical yarns

10

15

15

20

In a separate step, each yarn is passed over two sets of rolls and then the fully-drawn yarn is passed over a glass pin to a third set of rolls. Passage over the glass pin frictionally modifies the yarn and imparts latent crimp. Process conditions are given in Table III and properties of the pin-textured filaments are given in Table IV. The resultant crimp, while less than that obtained in Examples I, II and III with pin-textured polyester yarns, is sufficient to impart increased bulk to the polyamide yarn, which in turn improves tactile properties of fabrics such as tricot for slips, blouses and the like.

Table I

| Example No.                             | Pin-Texturing of Polyester Filaments of Examples I and II* |       |         |         |        |       |         |
|-----------------------------------------|------------------------------------------------------------|-------|---------|---------|--------|-------|---------|
|                                         | I                                                          | I     | I       | I       | I      | I     | II      |
| Sample No.                              | 1                                                          | 2     | 3       | 4       | 5      | 6     | —       |
| Polymer relative viscosity              | 22.0                                                       | 22.0  | 20.3    | 20.3    | (c)    | 15.0  | 19.5    |
| Drawing Step                            |                                                            |       |         |         |        |       |         |
| Feed roll speed, meters/min.            | 638                                                        | 638   | 638     | 638     | (d)    | 559   | 611     |
| Jet temperature, °C                     | 225                                                        | 225   | 210     | 185     | (d)    | 225   | 100     |
| Jet pressure, psig(kg/cm <sup>2</sup> ) | 85(6)                                                      | 85(6) | 98(6.9) | 60(4.2) | (d)    | 85(6) | 14.7(1) |
| Draw roll speed, meters/min.            | 2560                                                       | 2560  | 2533    | 2533    | 887(e) | 2561  | 1371    |
| Draw ratio                              | 4.0                                                        | 4.0   | 4.0     | 4.0     | (d)    | 4.6   | 1.94    |
| Pin-texturing step                      |                                                            |       |         |         |        |       |         |
| Yarn temperature, °C(a)                 | 42                                                         | 105   | R.T.    | 76      | R.T.   | 70    | ~0      |
| Pin type(b)                             | (1)                                                        | (1)   | (2)     | (2)     | (2)    | (1)   | (3)     |
| Tension before pin, g./fil.             | 5.1                                                        | 3.4   | (c)     | (c)     | (c)    | 3.1   | 1.8     |
| Tension after pin, g./fil.              | 7.2                                                        | 5.1   | (c)     | (c)     | (c)    | 5.4   | 4.1     |
| Tension change, g./fil.                 | 2.1                                                        | 1.7   | (c)     | (c)     | (c)    | 2.3   | 4.3     |
| Contact length, cm.                     | 0.5                                                        | 0.5   | 0.12    | 0.12    | 0.36   | 0.75  | 0.75    |
| Average velocity, cm./sec.              | 4308                                                       | 4371  | 4182    | 4290    | 1554   | 4346  | 2299    |
| Δ T max. parameter, °C                  | 216                                                        | 172   | (c)     | (c)     | 233    | 209   | 273     |
| Pulling roll speed, meter/min.          | 2612                                                       | 2686  | 2487    | 2615    | 978    | 2654  | 1388    |
| % stretch between draw & pull rolls     | 2                                                          | 5     | 0       | 3       | 10     | 3.6   | 1       |
| Windup speed                            | 2567                                                       | 2628  | (c)     | (c)     | 956    | 2612  | 1388    |
| Pin-textured yarn                       |                                                            |       |         |         |        |       |         |
| Denier                                  | 144                                                        | 141   | 71      | 72      | 70     | 127   | 130     |
| Number of filaments                     | 34                                                         | 34    | 34      | 34      | 34     | 34    | 34      |
| Break elongation, % (f)                 | 38.1                                                       | 34.5  | 30      | 31      | 36     | 28.4  | ~13.5   |
| Boil-off shrinkage, % (f)               | 16.8                                                       | 9.8   | 16.7    | 16.4    | 10     | 11.5  | ~17     |
| Break elongation, % (g)                 | 30.6                                                       | 28.4  | 32      | 30      | (c)    | 24    | 13.6    |
| Boil-off shrinkage, % (g)               | 17.7                                                       | 11.3  | 18.3    | 16.3    | (c)    | 11    | 17      |

\*Notes:

(a)R.T. = room temperature.

(b)Pin types identified in text.

(c)These parameters were not measured or calculated.

(d)Commercial yarn with fully drawn filaments is fed; drawing step is by-passed.

(e)Speed is removed from package.

(f)Filament properties before pin-texturing.

(g)Filament properties after pin-texturing.

before pin-texturing are as follows:

Table II

| A. Modified Portion of Filament <sup>(a)</sup>              | Pin-Textured Filaments of Examples I and II |      |      |      |      |      |      |
|-------------------------------------------------------------|---------------------------------------------|------|------|------|------|------|------|
|                                                             | I-1                                         | I-2  | I-3  | I-4  | I-5  | I-6  | II   |
| Thickness, microns                                          | 2.3                                         | 2.1  | 1.6  | 1.4  | 1.4  | 1.9  | 1.5  |
| Width % of filament diameter                                | 35                                          | 45   | 53   | 49   | 45   | 46.2 | 54.8 |
| Area occupied, % of fil. cross-section                      | 4.9                                         | 5.9  | 8.4  | 7.6  | 7.9  | 5    | 5.7  |
| Average length of discontinuities, mm.                      | 0.97                                        | 1.04 | 2.08 | 0.68 | 1.25 | 1.01 | 1.39 |
| Discontinuities longer than 2 mm.:                          |                                             |      |      |      |      |      |      |
| % of total number                                           | 0                                           | 0    | 25   | 0    | 7    | 0    | 18.7 |
| % of filament length                                        | 0                                           | 0    | 2    | 0    | 1    | 0    | 3.4  |
| B. Crimp Characteristics <sup>(b)</sup>                     |                                             |      |      |      |      |      |      |
| Average crimpes per 2.54 cm.                                | 43                                          | 55   | 41   | 39   | 34   | 34   | 49   |
| % of fil. length with more than:                            |                                             |      |      |      |      |      |      |
| 15 crimpes/2.54 cm.                                         | 99                                          | 100  | 100  | 99   | 100  | 100  | 100  |
| 20 crimpes/2.54 cm.                                         | 98                                          | 100  | 100  | 98   | 100  | 100  | 100  |
| Distribution of middle 90%, R <sub>5</sub> -R <sub>45</sub> | 40                                          | 25   | 33   | 27   | 21   | 15   | 19   |
| (R <sub>5</sub> -R <sub>45</sub> )/average                  | 0.92                                        | 0.45 | 0.8  | 0.69 | 0.62 | 0.44 | 0.39 |

Table II-continued

| A. Modified Portion of Filament <sup>(a)</sup> | Pin-Textured Filaments of Examples I and II |      |      |      |      |      |      |
|------------------------------------------------|---------------------------------------------|------|------|------|------|------|------|
|                                                | I-1                                         | I-2  | I-3  | I-4  | I-5  | I-6  | II   |
| Coefficient of variation, %                    | 27.1                                        | 13.1 | 22.8 | 21.5 | 18.3 | 12.6 | 11.9 |

## Notes:

<sup>(a)</sup>Measured before the heat relaxation treatment.<sup>(b)</sup>Measured after relaxation for 5 min. in air at 180°C.

I-2 and II are samples that were also jet-screen bulked.

Crimp is given in crimps per 2.54 cm. of filament length.

All crimp characteristics are normalized to 2.5 denier/filament.

Table III

| Example No.                                | Pin-Texturing of Filaments of Examples III and IV* |       |       |       |       |                |                |
|--------------------------------------------|----------------------------------------------------|-------|-------|-------|-------|----------------|----------------|
|                                            | III-A                                              | III-B | III-C | III-D | III-E | IV-A           | IV-B           |
| Polymer                                    | 2GT                                                | 2GT   | 2GT   | 2GT   | 2GT   | Nylon          | PACM-12        |
| Polymer, relative viscosity <sup>(b)</sup> | 22.0                                               | 22.0  | 22.0  | 22.0  | 22.0  | 45             | 40             |
| Drawing Step                               |                                                    |       |       |       |       |                |                |
| Feed roll speed, meters/min.               | 415                                                | 415   | 623   | 623   | 265   | 860            | 529            |
| Jet temperature, °C.                       | 225                                                | 225   | 225   | 225   | 225   | <sup>(d)</sup> | <sup>(d)</sup> |
| Jet pressure, psig/kg/cm. <sup>2</sup>     | 85(6)                                              | 85(6) | 85(6) | 85(6) | 85(6) | <sup>(d)</sup> | <sup>(d)</sup> |
| Draw roll speed, meters/min <sup>(c)</sup> | 1875                                               | 1875  | 2560  | 2560  | 1189  | 1189           | 1189           |
| Draw ratio                                 | 4.5                                                | 4.5   | 4.1   | 4.1   | 4.5   | 4              | 2.3            |
| Pin-Texturing Step                         |                                                    |       |       |       |       |                |                |
| Yarn temperature, °C. <sup>(d)</sup>       | 90                                                 | 90    | 92    | 92    | 60    | R.T.           | R.T.           |
| Pin type <sup>(d)</sup>                    | (3)                                                | (4)   | (1a)  | (1a)  | (4)   | (5)            | (5)            |
| Tension before pin, g/fil.                 | 2.5                                                | 3.2   | 2.5   | 0.9   | 2.5   | 0.3            | 4.4            |
| Tension after pin, g/fil.                  | 4.2                                                | 4.3   | 4.1   | 2.9   | 4.4   | 4.7            | 9.4            |
| Tension change, g/fil.                     | 1.7                                                | 1.1   | 1.6   | 2.0   | 1.9   | 4.4            | 5.0            |
| Contact length, cm.                        | 0.37                                               | 0.25  | 0.37  | 0.75  | 0.50  | 0.50           | 0.50           |
| Average velocity, cm./sec.                 | 3179                                               | 3179  | 4374  | 4310  | 2001  | 1981           | 1974           |
| Δ T Max. parameter, °C.                    | 183                                                | 150   | 207   | 184   | 141   | 272            | 219            |
| Pulling roll speed, meters/min.            | 1939                                               | 1939  | 2688  | 2612  | 1212  | 1189           | 1180           |
| % stretch between draw & pull rolls        | 3.4                                                | 3.4   | 5     | 2     | 2     | 0              | -0.8           |
| Windup speed, meters/min.                  | 1903                                               | 1903  | 2633  | 2560  | 1179  | 1189           | 1180           |
| Pin-textured yarn:                         |                                                    |       |       |       |       |                |                |
| Denier                                     | 123                                                | 123   | 123   | 124.5 | 127.5 | 131            | 258            |
| Number of filaments                        | 34                                                 | 34    | 34    | 34    | 34    | 34             | 34             |
| Break elongation, % <sup>(b)</sup>         | 30.2                                               | 28.6  | 29.4  | 32.2  | 34.2  | <sup>(e)</sup> | <sup>(e)</sup> |
| Boil-off shrinkage, % <sup>(b)</sup>       | 12.7                                               | 11.8  | 13    | 12.1  | 14.1  | <sup>(e)</sup> | <sup>(e)</sup> |
| Break elongation, % <sup>(b)</sup>         | 24.9                                               | 24.1  | 28.0  | 31.5  | 24.9  | 22             | <sup>(e)</sup> |
| Boil-off shrinkage, % <sup>(b)</sup>       | 11.3                                               | 11.6  | 12.0  | 11.0  | 10.3  | 10             | 7              |

## \*Notes:

<sup>(a)</sup>R.T.=room temperature.<sup>(b)</sup>Pin type identified in text.<sup>(c)</sup>These parameters were not measured.<sup>(d)</sup>Not used for polyamide filaments.<sup>(e)</sup>The nylon feed yarn of IV-A was previously fully drawn and had a 1.4X recoverable stretch.<sup>(f)</sup>Measured in a solution of 0.5 g. of polymer in 100 c.c. of Fomal for Ex. IV-A and IV-B.<sup>(g)</sup>filament properties before pin-texturing.<sup>(h)</sup>filament properties after pin-texturing.

Table IV

| A. Modified Portion of Filament <sup>(a)</sup>              | Pin-Textured Filaments of Examples III and IV* |       |       |       |       |                |                |
|-------------------------------------------------------------|------------------------------------------------|-------|-------|-------|-------|----------------|----------------|
|                                                             | III-A                                          | III-B | III-C | III-D | III-E | IV-A           | IV-B           |
| Thickness, microns                                          | 2.9                                            | 2.1   | 1.8   | 1.8   | 1.6   | <sup>(d)</sup> | <sup>(d)</sup> |
| Width, % of filament diameter                               | 46.3                                           | 48.7  | 43.5  | 41.0  | 34.2  | <sup>(d)</sup> | <sup>(d)</sup> |
| Area occupied, % of fil. cross section                      | 7.5                                            | 5.6   | 5.1   | 4.7   | 3.3   | <sup>(d)</sup> | <sup>(d)</sup> |
| Average length of discontinuities, mm.                      | 0.87                                           | 0.58  | 0.84  | 0.73  | 0.72  | 1.1            | <sup>(d)</sup> |
| Discontinuities longer than 2mm.:                           |                                                |       |       |       |       |                |                |
| % of total number                                           | 0                                              | 0     | 0     | 0     | 0     | 5              | <sup>(d)</sup> |
| % of filament length                                        | 0                                              | 0     | 0     | 0     | 0     | 0.5            | <sup>(d)</sup> |
| B. Crimp Characteristics <sup>(b)</sup>                     |                                                |       |       |       |       |                |                |
| Average crimps per 2.54 cm.                                 | 34                                             | 41    | 29    | 27    | 27    | 22             | 14             |
| % of fil. length with more than:                            |                                                |       |       |       |       |                |                |
| 15 crimps/2.54 cm.                                          | 100                                            | 99    | 100   | 100   | 97    | 98             | 32             |
| 20 crimps/2.54 cm.                                          | 100                                            | 99    | 99    | 96    | 93    | 76             | 0              |
| Distribution of middle 90%, R <sub>5</sub> -R <sub>95</sub> | 14                                             | 16    | 15    | 13    | 14    | 9              | 9              |
| (R <sub>5</sub> -R <sub>95</sub> )/average                  | 0.41                                           | 0.39  | 0.52  | 0.48  | 0.52  | 0.39           | 0.64           |
| Coefficient of variation, %                                 | 11.3                                           | 12.0  | 13.0  | 13.8  | 16.2  | 10.7           | 16.0           |

## \*Notes:

<sup>(a)</sup>Measured before the heat relaxation treatment.<sup>(b)</sup>Measured after relaxation for 5 min. in air at 180°C Crimp is given in crimps per 2.54 cm. of filament length. All crimp characteristics are normalized to 2.5 denier/filament.<sup>(c)</sup>These parameters were not measured or calculated.<sup>(d)</sup>The tests for these parameters were not applicable.

## We claim:

1. In the process for preparing multifilament yarn of filaments which crimp due to asymmetric shrinkage

when relaxed, wherein a yarn bundle of filaments spun from a single synthetic linear organic thermoplastic polymer is passed in contact with a heated surface to

21

provide asymmetric shrinkage properties on opposite sides of filaments, the improvement which comprises (a) drawing the filaments to provide the approximate break elongation desired in the product and (b) passing the drawn filaments at high speed in frictional contact with a durable, wear-resistant surface under frictional tension sufficient to generate all of the heat required to provide the desired asymmetric shrinkage properties without otherwise heating the wear-resistant surface.

2. A process as defined in claim 1 wherein the drawn filaments are passed in frictional contact with the durable, wear-resistant surface at a speed of at least 900 yards per minute.

3. A process as defined in claim 2 wherein the filament speed is 1,000 to 4,500 yards per minute.

4. A process as defined in claim 3 wherein the durable, wear-resistant surface is provided by a cylindrical pin 3 to 10 millimeters in diameter.

5. A process as defined in claim 4 wherein the filaments contact the pin over an arc of 30° to 180°.

6. A process as defined in claim 2 wherein the filament speed is at least 2,000 yards per minute.

7. A process as defined in claim 1 wherein the filaments are drawn to have a boil-off shrinkage of 5 to 25 percent when determined prior to step (b).

8. A process as defined in claim 1 wherein the filaments are drawn to have 15 to 40 percent elongation at break and 8 to 16 percent boil-off shrinkage.

9. A process as defined in claim 1 wherein the drawn filaments are fed from step (a) to step (b) at a temperature of 25° to 100°C.

10. A process as defined in claim 1 wherein the tension on the filaments immediately after contact with the wear-resistant surface minus the tension immediately before the surface is 0.7 to 7 grams per filament for filaments of 1.5 to 10 denier.

11. A process as defined in claim 10 wherein said tension difference is 1 to 2 grams per filament and the filaments are composed of a polyester.

12. A process as defined in claim 1 wherein the filaments are in frictional contact with the surface for a distance of 0.5 to 15 millimeters.

13. A process as defined in claim 1 wherein the filaments are in frictional contact with the surface for a distance of 1 to 10 millimeters.

14. A process as defined in claim 1 wherein the temperature rise calculated by the following formula is 100° to 300°C.:

$$\Delta T_{\max} = 0.0283 (f_2 - f_1) \sqrt{\frac{V}{Lkcd}}$$

22

where  $f_1$  and  $f_2$  are the average tensions on the filaments immediately before and after frictional contact with the wear-resistant surface, in grams per filament;  $V$  is the average speed of the filaments contacting the surface, in centimeters per second;  $L$  is the frictional contact length between the filaments and the surface, in centimeters;  $k$  is the thermal conductivity of the filaments, in cal./cm.sec.°C.;  $d$  is the specific heat of the filaments, in cal./g.°C.; and  $d$  is the denier per filament.

15. A process as defined in claim 1 wherein the wear-resistant surface is a curved surface.

16. A process as defined in claim 1 wherein the wear-resistant surface is the surface of a ceramic pin.

17. A process as defined in claim 1 wherein the filaments are composed of a polyamide.

18. A process as defined in claim 1 which is a coupled spin/draw/pin-texturing process wherein the yarn is drawn to have 15 to 40 percent break elongation and 8 to 16 percent boil-off shrinkage.

19. A process as defined in claim 1 wherein the filaments are composed of polyethylene terephthalate.

20. A process for treating multifilament yarn to impart asymmetric shrinkage properties to drawn yarn filaments of denier per filament ( $d$ ) and consisting of a single synthetic linear polyester composition, which comprises passing the drawn filaments at a high speed ( $V$ ) in frictional contact with an unheated ceramic pin for a frictional contact length ( $L$ ) of 0.05 to 1.5 centimeters under tension conditions which apply a filament stretch of 2 to 5 percent, said pin having a coefficient of friction of 0.2 to 1.2 and said filaments having a temperature of 25° to 100°C. just prior to contact with the pin, the values of said variables being such that the temperature rise calculated by the following formula is at least 140°C.:

30

35

$$\Delta T_{\max} = 2.26 (f_2 - f_1) \sqrt{\frac{V}{Ld}}$$

40

where  $f_1$  and  $f_2$  are the average tensions on the filaments immediately before and after frictional contact with the pin.

45

21. A process for treating the filaments of a multifilament yarn as defined in claim 20, wherein said yarn has been drawn to have an elongation of 15 to 40 percent and a boil-off shrinkage of 8 to 16 percent before the yarn filaments are passed in contact with said pin.

\* \* \* \* \*

55

60

65